

CATION OF TEXTILES &amp; FIBERS,

## UNITED STATES PATENT OFFICE.

ANDREW POULSON, OF WIDNES, ENGLAND.

BLEACHING, SCOURING, AND DECORTICATING FABRICS OR FIBROUS MATTER.

1,254,727.

Specification of Letters Patent. Patented Jan. 29, 1918.

No Drawing.

Application filed February 12, 1917. Serial No. 148,291.

*To all whom it may concern:*

Be it known that I, ANDREW POULSON, a subject of the King of Great Britain, residing at Springfield Villa, Hough Green, 5 Widnes, England, have invented certain new and useful Improvements in Bleaching, Scouring, and Decorticating Fabrics or Fibrous Matter, of which the following is a specification.

10 This invention relates to an improved process and composition for bleaching textile fabrics or other material, such as waste paper, straw board, or the like, and for scouring or decorticating wool or other fibrous 15 material and is designed to provide a more economical process than those at present obtaining for such purposes. The present usual process of bleaching consists in immersing the material to be bleached in a 20 tank or the like containing a solution of sodium hypochlorite, or bleaching powder, together with some suitable acid the solution being kept at boiling point for from eight to twelve hours, after which the material 25 is removed and washed, in some cases with a solution of weak acid or soap and water.

According to this invention the material to be bleached is boiled in a tank or the like 30 receptacle for from one to two hours, in a solution of a special powder, consisting of about equal parts of ordinary commercial washing soda and of sodium bicarbonate, the solution being made up approximately in 35 the proportions of one ounce of such powder per gallon of water. After the material has been boiled for the period mentioned and while the solution is still boiling a small portion, say, about three per cent. of a 40 solution of sodium hypochlorite is added to the solution in the receptacle, and the combined solution boiled for another one to two hours. The bleaching operation is then completed and the material may be removed and 45 dried or treated in any suitable manner. If desired the sodium hypochlorite instead of being made up as a separate solution, may be incorporated with the washing soda and sodium bicarbonate in the first instance.

50 Such a process results in a considerable economy in the time requisite for effecting the bleaching operation, and is found to be

in no wise detrimental to the fibrous character of the material being treated. Further, the one operation of boiling serves to wash 55 as well as bleach the fabric or other material, and the additional expense necessitated by having separate washing baths, as in the usual process, is avoided. The process is found to be quite effective for bleaching ordinary brown paper, for removing printer's ink from old newspapers, and for the ordinary bleaching requirements of the textile industries.

The powder consisting of equal parts of 60 commercial washing soda or soda ash and of sodium bicarbonate may be used in weak solution for ordinary washing purposes or as a cleanser for paint or varnish. By making the powder up into a very strong solution, flax, hemp, jute and other fibers may be decorticated or retted in a few hours, thus securing a considerable saving over the 65 present methods of dealing with such fibrous material which require them to be left for a 70 considerable time to rot, thus necessarily 75 weakening the fibers.

The powder is also of great value as a purifier and preservative for fish, hams and other foods, which have become high or 80 rancid, while as a meat preservative in hot weather it has been found superior to borax or boracic acid. For scouring raw wool in bulk and for cleaning it of its impurities, a 85 solution of the powder is found very effective, the wool besides being cleaned and scoured having all the fats removed and rendered down.

I claim—

The improved process for bleaching textile fabric or other material, which consists in boiling the material to be bleached in a solution of commercial washing soda and sodium bicarbonate so as to soften the 90 gummy material therein, and subsequently 95 adding a small quantity of sodium hypochlorite to the solution containing the fabric, and a continuation of the boiling.

In testimony whereof I affix my signature in presence of two witnesses.

ANDREW POULSON.

Witnesses:

A. J. DAVIES,  
J. M. CORMICK.

Copies of this patent may be obtained for five cents each, by addressing the "Commissioner of Patents, Washington, D. C."

401  
X420.1